

May 17, 1927.

1,629,185

F. J. TONE

NONSLIP FLOOR CONSTRUCTION

Filed Jan. 25, 1922

*Fig.1.*



*Fig.2.*



INVENTOR  
*Frank J. Tone*

by *Byrnes, Stetson, Byrnes & Carmel*  
*his Attorneys*

## UNITED STATES PATENT OFFICE.

FRANK J. TONE, OF NIAGARA FALLS, NEW YORK, ASSIGNOR TO THE CARBORUNDUM COMPANY, OF NIAGARA FALLS, NEW YORK, A CORPORATION OF PENNSYLVANIA.

## NONSLIP FLOOR CONSTRUCTION.

Application filed January 25, 1922. Serial No. 531,772.

Figure 1 is a perspective view of a non-slip floor unit or block; and

Figure 2 is a similar view of a broken fragment of floor; both constructed in accordance with my invention.

My invention relates to non-slip floor surfaces, wearing surfaces, stairway treads and the like; particularly those in which the wearing surface contains abrasive material.

10 The object of my invention is to reduce the cost of such surfaces without affecting the appearance or qualities thereof.

In carrying out my invention, I first form a molded plate or slab consisting of abrasive grains united by a binder to form a slab. The abrasive grains may consist of silicon carbide, aloxite (which is a form of artificial corundum) or other hard and sharp material. The grains may be of graded, selected sizes or mixtures of sizes to meet the conditions. The grains are united to form the slab by means of any suitable binder, such as one of a ceramic cement, or other suitable character.

15 As a typical example, I will describe the use of silicon carbide grains with a ceramic binder for making the preliminary slab or plate. A mixture is made of the following composition:

20 Silicon carbide grains in a mixture of sizes from No. 30 to No. 180, 76 parts; feldspar, 18 parts; kaolin, 6 parts. This is moistened with water to the consistency of molding sand and then molded in presses to the

25 form of thin plates or slabs of any suitable thickness. For the purpose of ordinary interior floors, I prefer a thickness of from  $\frac{1}{8}$  to  $\frac{1}{4}$  of an inch.

Instead of molding in iron molds under 30 hydraulic pressure, it may be found desirable in some cases to use an extruding press from which a continuous plate or slab is forced. The dimensions of the plates or slabs are not important, and they may be of any size convenient for molding and burning. After molding, the pieces are dried and burned in a kiln at a temperature of approximately  $1300^{\circ}$  C., at which point the bond vitrifies and unites the abrasive grains 35 into a hard unitary mass.

After burning, the slabs are broken up into irregular fragments ranging from  $\frac{1}{4}$  of an inch to 1 inch in size, each fragment, of course, having two shaped or molded surfaces, the other surfaces being irregular in

outline. In this step of breaking up, corrugated rolls or any other convenient means may be employed.

In forming the flooring by the use of these fragments, I preferably form a solid base or main supporting body of Portland cement or other cementitious material. This foundation is then preferably covered with a layer of about  $\frac{7}{8}$  of one-to-three cement mortar, and the non-slip fragments 60 are laid on this cement layer with their flat molded surfaces uppermost. They are placed in irregular order and with small irregular spaces between the fragments so that the finished plate has the appearance of terrazzo. After the pieces are laid, they are tamped down and preferably leveled. After setting, they are preferably grouted in with cement and the surfaces may then be finished off by grinding to a plane surface 70 75 with a grinding wheel, rubbing block or other suitable means.

In applying the pieces, they may be, laid by hand, or they may be first fastened to a paper backing in the well known manner of laying mosaic floors. In the latter case, the pieces are laid on the wet cement surfaces with the free surface down and the paper side up. They may then be pressed down into the plastic cement by means of surface boards or rollers, and after setting, the paper is soaked off. They are then grouted with cement and brought to a finished surface.

80 In the above example, I have described the making of flooring having a surface composed of carborundum pieces. This gives a floor of dark uniform color. But it is evident that many modifications may be made by using different varieties of abrasives or 85 by using different kinds and colors of the pieces, and different colors of bonding material may also be used to give variegated colors and effects. For this purpose I may use aloxite and may employ different colored 90 porcelains and vitreous bodies, in which smaller percentages of the abrasive are incorporated for non-slip purposes, the color being masked to a certain extent by the bonding material.

95 The advantages of my invention will be obvious to those skilled in the art since by first forming a molded slab or plate, which is then broken up and the pieces inserted in the floor unit or floor, a minimum of 100 105 110

abrasive is required, this being the expensive part of the material. By having the pre-molded surface or surfaces, much surface grinding and polishing is saved. In this respect, the flooring is much cheaper than the terrazzo type. The irregular shaped pieces are much cheaper to produce than ordinary mosaic, in which each piece must be separately molded, and the cost of molding and burning is considerably higher.

Many variations may be made in the abrasive material, the binder, the method of making the preliminary slab or plate, the manner of breaking the slab, etc., without departing from my invention.

I claim:

1. A non-slip floor surface including a supporting mass of cement having plane-faced fragments of a flat slab of abrasive material embedded in the upper surface thereof to a uniform depth and with the plane upper faces of the fragments substantially flush with the surface of the mass in which they are embedded and exposed to present a tread surface.
2. A non-slip floor surface including a supporting mass of cement having plane-faced irregular fragments of a flat slab of

abrasive material embedded in the upper surface thereof to a uniform depth and with the plane upper faces of the fragments substantially flush with the surface of the mass in which they are embedded and exposed to present a tread surface, the said fragments being non-uniformly scattered over the surface in relatively close proximity to each other.

3. The method of forming a non-slip floor which consists in forming abrasive material into slabs having substantially flat faces and of substantially uniform thickness, shattering such slabs to obtain irregular substantially flat-faced fragments of substantially uniform thickness, and then embedding such fragments to a substantially uniform depth in a plastic cementitious mass with one of the substantially flat faces of each piece exposed and substantially flush with the cementitious mass, and with the most of the fragments out of contact with other fragments whereby the cementitious material surrounds the fragments to firmly secure them in place.

In testimony whereof I have hereunto set my hand.

FRANK J. TONE.